

J. E. JOHNSON, JR.  
PROCESS OF TREATING CAST IRON.  
APPLICATION FILED DEC. 8, 1913.

1,150,201.

Patented Aug. 17, 1915.



Attest:  
M. R. Manning  
W. J. Dolan

Inventor:  
J. E. Johnson Jr.  
by  
Rogers, Kennedy & Campbell Atty's.

# UNITED STATES PATENT OFFICE.

JOSEPH E. JOHNSON, JR., OF NEW YORK, N. Y.

## PROCESS OF TREATING CAST-IRON.

1,150,201.

Specification of Letters Patent. Patented Aug. 17, 1915.

Application filed December 8, 1913. Serial No. 805,251.

To all whom it may concern:

Be it known that I, JOSEPH E. JOHNSON, Jr., a citizen of the United States, residing at New York, in the county of New York and State of New York, have invented certain new and useful Improvements in Processes of Treating Cast-Iron, of which the following is a specification, reference being had therein to the accompanying drawing.

10 This invention relates to the treatment of cast iron, and it consists in a process for removing oxygen therefrom in order that the iron may be free from chilling properties, and will possess a soft and highly graphitic 15 nature, characteristics which I have found desirable for certain purposes for which cast iron is used.

I have discovered that the chilling properties possessed by certain cast irons are 20 due mainly to the presence of oxygen therein, the oxygen tending to cause the carbon to take the combined rather than the graphitic condition, and causing the graphite formed when the metal cools, to take the 25 form of nodules rather than that of flakes.

For certain purposes it is very desirable that the iron be of this structure, but for other purposes for which cast iron is used, such structure of the iron is objectionable 30 and therefore it is desirable to remove the oxygen so that the iron will not only be free from chilling properties but the graphite will take the form of flakes, these two conditions conduced to softness of the iron.

35 In the removal of the oxygen, which is the aim of my invention, I take advantage of the chemical reactions which will occur between oxygen and other constituent elements of the iron, such as silicon and carbon, 40 under temperature conditions considerably higher than the temperature at which the iron comes from the furnace, and while subjecting a bath of the molten iron to such temperature conditions, I, in accordance 45 with my invention, maintain such a condition above the surface of the bath, that oxygen will be prevented from entering the bath at this point. As a result of this proceeding, the oxygen will be effectually re- 50 moved, leaving the iron free from chilling qualities and the graphite in flaky form.

In the accompanying drawings I have shown an electric furnace of the induction type which I find preferable for carrying 55 my process into practice.

In the practice of the process I heat a bath A of cast iron in an electric furnace B constructed with a chamber or space b above the surface of the bath the purpose of which will presently appear. The degree of heat given the bath is such as to promote reactions between the oxygen and other constituent elements of the iron, particularly silicon and carbon, the oxygen combining with the silicon and forming silica 60 which will float on the surface of the bath, and combining also with the carbon of the bath, thereby forming CO gas which will leave the bath in the form of bubbles. The temperature which I find necessary to promote these reactions, is considerably above that of the iron when it is tapped from the coke furnace, and should be as high as 3000° F. or thereabout. During the heating of the 70 bath and while the above mentioned reactions are taking place, I maintain above the surface of the bath, such a condition that oxygen will be prevented from entering the metal from the outside. Preferably this condition is brought about by giving the 75 atmosphere above the bath a reducing quality, by injecting into the chamber b, any desired quantity of CO gas even as high as 100% of the same. Or hydrogen gas may be employed for this purpose, or 80 any of the many hydro-carbon gases. Such gas may be so introduced into the chamber b, as to force out the atmospheric air and products of the reactions taking place in the bath, the effect of which will be to maintain above the surface of the bath, a condition of atmosphere which will prevent the entrance of oxygen into the bath.

By the employment of an electric furnace for heating the bath, the degree of heat obtainable is under absolute control, and does not depend upon the atmosphere above the bath, which in other types of heating furnaces must have a composition based on the temperature to be produced, rather than on the effect desired on the bath. By the use of the electric furnace therefore the bath may be heated to a degree high enough to bring about the desired reactions of the constituent elements of the bath and resulting in the removal of the oxygen to the final traces, while at the same time the condition existing above the surface of the bath, may be so controlled that there will be no possibility of oxygen entering the bath at this 105 110

point or externally. While such conditions may be brought about as above stated by introducing into the space above the bath, an atmosphere of a reducing quality, it may also be brought about by creating a vacuum in the chamber *b*, the essential feature in this respect being the maintaining of such a condition above the bath, that no oxygen from external sources can enter therein. While an induction type of electric furnace is shown as the preferable type for carrying my invention into effect, the process may be carried out also by the use of an electrode furnace, but because of the high conductivity of such baths, the size of the electrodes would be unduly large, and therefore such furnace would not be as suitable as that shown. It will be understood therefore that my improved process is not limited in its practice to the particular type of furnace shown, but may be carried into effect by any means by which the results described above are brought about.

Having thus described my invention what 25 I claim is:

1. The process of removing oxygen from cast iron, which consists in heating a bath of said iron to a temperature high enough to promote reaction between the oxygen and other constituents of the bath, while maintaining a condition above the bath which will prevent the entrance of oxygen therein.
2. The process of removing oxygen from cast iron, which consists in heating a bath 35 of said iron in the presence of a reducing atmosphere to a temperature high enough to promote reaction between the oxygen and other constituents of the bath.
3. The process of removing oxygen from 40 cast iron, which consists in heating a bath of said iron to a temperature above that at which the metal comes from the furnace, such temperature being high enough to promote reaction between the oxygen and other constituents of the bath, while maintaining

a condition above the bath which will prevent the entrance of oxygen therein.

4. The method of removing oxygen from cast iron, which consists in heating a bath of said iron in an electric furnace to a temperature which will promote reaction between the oxygen and other constituents of the bath, said heating being carried on under conditions which will prevent the entrance of oxygen into the bath.

5. The method of removing oxygen from cast iron, which consists in heating a bath of said iron in an electric furnace to a temperature well above that at which the iron comes from the coke furnace, such temperature being high enough to promote reaction between the oxygen and other constituents of the bath, and maintaining over said bath an atmosphere of a reducing nature to prevent the entrance of oxygen into the bath.

6. The method of removing oxygen from cast iron, which consists in heating a bath of said iron in an electric furnace to a temperature well above that at which the iron comes from the coke furnace such temperature being high enough to promote reaction between the oxygen and other constituents of the bath, while maintaining such a condition above the bath that oxygen will be prevented from entering therein.

7. The method of removing oxygen from cast iron, which consists in heating a bath of said iron to a temperature sufficient to promote reactions between the oxygen, silicon and carbon of the bath, while maintaining such a condition above the bath that the entrance of oxygen therein will be prevented.

In testimony whereof I have affixed my signature in presence of two witnesses.

JOSEPH E. JOHNSON, Jr.

Witnesses:

Wm. J. DOLAN,  
W. R. KENNEDY.

Copies of this patent may be obtained for five cents each, by addressing the "Commissioner of Patents,  
Washington, D. C."